

June 12, 1934.

C. L. KELLER

1,962,660

CARTON AND METHOD OF SEALING IT

Filed March 23, 1929



*Fig. 1.*



INVENTOR.  
*Charles L. Keller*  
BY  
*Allen & Allen*  
ATTORNEYS.

Patented June 12, 1934

1,962,660

# UNITED STATES PATENT OFFICE

1,962,660

## CARTON AND METHOD OF SEALING IT

Charles L. Keller, Cincinnati, Ohio, assignor to  
The Richardson Company, Lockland, Ohio, a  
corporation of Ohio

Application March 23, 1929, Serial No. 349,477

4 Claims. (Cl. 93—36)

My invention is addressed to the manufacture and sealing of cartons from blanks of board which have been treated with paraffin, wax, oils or the like substances to render them water-  
proof and grease resistant. Inasmuch as it is not practical to coat cartons with these substances after the cartons have been folded and glued into shape for shipment, due to the danger of sticking the parts of the folding carton together by the paraffin, the general difficulty in handling folding cartons which have already been glued, and the difficulties to be met with in gaining the proper surface finish upon the paraffin layer, it has uniformly been the practice to manufacture paraffined cartons by printing, cutting and scoring a blank of suitable board, paraffining this cut out carton, and then removing the paraffin from the glue flap and the portion of the side of the carton to which the glue flap is to be stuck. This last step is necessary because the adhesives heretofore thought applicable for the pasting of folding cartons will not adhere to a paraffined surface. Various methods have been proposed for removing the paraffin, such as passing the desired portions of the carton blank over hot plates, scraping or cutting the paraffin off with or without the application of heat, impinging jets of steam upon the desired portion so as to drive the paraffin into the board, and the like. All of these expedients are somewhat cumbersome and require additional equipment.

Again, paraffined cartons have been restricted to folding cartons of the tuck end type. The 35 carton manufacturer can glue the knock down blank in the factory, but ordinarily the user is not able to practice the same methods in sealing these cartons. Consequently paraffined cartons have had to be made of the tuck end type; 40 and where a water tight seal was desired in a type of carton in which the sealing flaps are glued, it has been the general practice to use an unparaffined shell filled and glued in the usual manner and then covered with a heat 45 sealed wax paper wrapper. The use of the means hitherto proposed for removing the paraffin from those portions of a carton to which glue is intended to bond, would result in impairing the surface finish of the paraffin over 50 those portions. If the portions were of comparatively large size, as for example the end sealing flaps of cartons, the appearance of the completed and sealed carton would be greatly impaired. A still greater objection to the use 55 of the above methods is that extra machines

and handling are required to remove paraffin from flaps in more than one direction. Indeed, to date, no such machine is in general use.

It is an object of my invention to provide an adhesive which will adhere to a paraffined surface and consequently a method of gluing knock down carton blanks without the necessity of the provision of means for removing paraffin or wax from any portions thereof.

It is an object of my invention to provide a glued knock down carton blank in which the original water- and greaseproofness has been preserved and has not been impaired over any area by a method employed to remove paraffin or wax therefrom.

It is still another object of my invention to provide a paraffined folding carton or other type of paraffined carton with sealing flaps, and a method of sealing such cartons after they have been filled, the method not involving the necessity for the removal of paraffin or wax from any surfaces prior to the application of glue thereto. It is to be noted that paraffin itself has been used as a seal, and consequently in part at least as an adhesive, particularly in making the wax 80 wrappers mentioned above; but the binding effect of paraffin is too weak to permit the satisfactory manufacture of cartons by any such practice. The band of adhesive along the glued flap in a carton blank is necessarily narrow and 85 must be quite strong. While somewhat less difficulty might be experienced in sealing the end flaps of a carton with paraffin alone, nevertheless this has not been regarded as practicable in a carton structure which forms the sole container for the material being shipped. In all cases where paraffin has been used as a sealing medium, of which applicant has knowledge, separate waxed wrappers or the equivalent have 90 been used over the cartons, and the wrappers 95 themselves have been heat sealed with paraffin.

These and other objects of my invention I accomplish by that certain process of which I shall now describe an exemplary embodiment.

In the drawing: Fig. 1 is a perspective view 100 of a carton to which my invention is applied; and Fig. 2 is a sectional perspective view of the same.

Broadly my invention comprises the provision of an adhesive which will adhere to a paraffined surface either by amalgamation with the paraffin or otherwise. An exemplary type of such an adhesive is asphaltum applied hot so that it fluxes with the paraffin, and effects a bond thereto which is at least as strong, and in prac- 110

tice may be stronger, than the internal strength of the board itself. This bond may be of two kinds. The preferable one is where the hot asphalt fluxes with the paraffin and penetrates to the actual surface of the board, so that pressure on the gluing machine permits only a very thin layer of asphalt-paraffin flux to remain and yield a fiber to fiber bond as strong or stronger than the paper itself. A less preferable, 10 but still practical, bond results when a thicker layer of asphalt remains so that, although it may penetrate to the surface of the bond, a fracture of the bond results in splitting the asphalt itself.

If the adhesive is an asphaltic substance, it is 15 used hot and it may be that beside the fluxing action noted above, the hot application of bituminous substance tends in some measure to drive the paraffin into the board. It is to be noted however, that whatever action occurs, over the 20 surface upon which the paraffin has thus been treated, there lies a film of bituminous substance which is also waterproof and grease-resistant, so that the proofness of the board is in nowise impaired.

25 My invention is not however restricted to the use of asphalt, but embraces any equivalent substance which has the characteristic of amalgamating with the paraffin which overlies the carton surface, and forming either by itself or 30 with the paraffin, an adhesive layer of the required strength. It embraces an adhesive which has the characteristic of penetrating through the paraffin layer and fastening on to the surface of the material to be pasted. Its usefulness is not 35 restricted to the gluing of paraffined cartons but has application wherever it is desired to stick together by adhesive action, two substances, at least one of which has previously been treated 40 with paraffin or wax. Thus it has application to the manufacture of bags, pouches and all manner of containers for hygroscopic goods, or goods which it is desired to seal in shipment against the effects of moisture, gases, grease and the like.

45 In an exemplary practice under my invention I employ as an adhesive an asphalt with Ball and Ring melting point of 150 to 160 degrees F., penetration 100 grams, 5 seconds of around 20. This is an asphalt commonly used for saturating 50 felt for felt base floor covering. I introduce this asphalt into the glue pot of a standard gluing machine, the glue pot, as in standard practice, being equipped with heating means generally of electric character. I run my adhesive quite hot, 55 say at 400-450° F. and I apply it to the cartons in the ordinary manner. Thus it will be seen that the practice of my invention makes no change excepting in the nature of the adhesive and in the temperature at which it is kept, over 60 ordinary practices in the gluing of carton blanks to form knock down folding cartons; nor are any additions to the gluing machine required, such as means separately to remove from the 65 surfaces to be glued, their coating of paraffin or wax. Some care has to be taken with my process to see that after the application of the bituminous adhesive to one surface, that surface is pressed into contact with the surface to which it is to be glued, before the adhesive has lost its tackiness; and it is usually advisable to employ some care in temperature control to prevent the dulling of the paraffin surfaces which fall adjacent in any stage of the gluing operation to the 70 heated band of adhesive. It goes without saying 75 that the amount of adhesive should be con-

trolled, just as in ordinary gluing, to the end that there may be no excesses to be squeezed out upon the carton surfaces. It is to be pointed out also that in some cases and with certain materials, I may use a solvent if desired in connection with my bituminous adhesive, and to the extent of the solvent used, dispense with the use of heat.

80 In these descriptions the term "glued" means the combining or pasting together of portions of paper or paper board cartons or containers with heat liquefiable or softenable adhesive material such as asphalt, pitch, gums, resins, etc., and in the manner of and with the equipment ordinarily used for this purpose with water soluble adhesive such as animal or destrin glues 85 and the like.

90 Other examples comprises the use at 400 degrees F. of an air blown asphalt of a 200 to 215 degrees F. Ball and Ring melting point, penetration 77 degrees F., 100 grams, 5 seconds of 20 to 25, made from Mexican or Mexican and Illinois crude; the use at 500 degrees F. of fatty acid pitch of Ball and Ring melting point 145 to 150 degrees F., penetration 77/100/5 of around 100 60; the use at 300 to 325 degrees F., of Montan wax; the use at 420 degrees F. of orange flake shellac; the use of Carnauba wax at 320 degrees F.; the use of sulphur at 265 degrees F.; the use at 300 degrees to 325 degrees F. of coal 105 tar pitch with 160 to 170 degrees F. Ball and Ring melting point; etc. The kind of bitumen to be used for paraffined cartons will vary with the purpose to which the carton is applied. An ice cream carton, for example, requires a type 110 of bituminous adhesive that will not open up at cold or freezing temperatures; a butter carton will not be frozen nearly so stiff; a cheese container may or may not be subjected to very low temperatures; a coconut (shredded) carton 115 never is frozen or chilled intentionally. Consequently, for those cartons never chilled nor frozen the 20 penetration steam refined asphalt or 25 penetration air blown asphalt will serve as an adhesive at room temperatures but will 120 not hold a good bond at cold temperatures. For the chilled cartons a fatty acid or stearine pitch will hold the bond at low temperatures, (if desired a flux of asphalt and stearine or other suitable bitumen can be used).

125 A typical soft fatty acid pitch is one with Ball and Ring melting point 130-135 deg. F., penetration 77/100/5 of 68, 32/200/60 of 29, 115/50/5 and is quite soft.

130 In the sealing of cartons after filling, the practice of my invention will comprise the substitution of my type of adhesive for other types of adhesive, the application thereof by the same means as at present employed, and the control 135 of temperature as outlined above in connection with the pasting of knock down carton forms.

Having thus described my invention, what I claim as new and desire to secure by Letters Patent, is:—

140 1. That process of forming and sealing cartons of paperboard having a surface layer of wax, which comprises superposing the parts thereof which are to be joined adhesively with mutually facing surfaces, at least one of which surfaces 145 has the wax layer, and, without previous removal of said wax, cementing said parts together by the application of hot bitumen, miscible to some extent at least with said wax, and thereby 150 permeating the wax surface layer, and having

greater adhesive and cohesive properties than said wax.

2. That process of forming or sealing cartons of paperboard having a surface layer of wax, which comprises superposing the parts thereof which are to be joined adhesively with mutually facing surfaces, at least one of which surfaces has the wax layer, and, without previous removal of said wax, cementing said parts together by the application of hot asphalt to said mutually facing surfaces.

3. A carton formed of paperboard having a surface layer of wax, at least two overlapping portions of the body of said carton with mutually facing surfaces, at least one of which

surfaces has the wax layer, being adhesively joined together by a bitumen which permeates the wax layer and directly contacts both surfaces of said paperboard, and which has greater adhesive and cohesive properties than said wax. 80

4. A carton formed of paperboard having a surface layer of wax, at least two overlapping portions of the body of said carton with mutually facing surfaces, at least one of which surfaces has the wax layer, being adhesively joined together by asphalt which permeates the wax layer and directly contacts both surfaces of said paperboard. 85

CHARLES L. KELLER.

90

95

100

105

110

115

120

125

130

135

140

145

150